# EUROPEAN PATENT SPECIFICATION

(11) **EP 1 311 352 B1**
(45) Date of publication and mention of the grant of the patent: **18.05.2005**
(21) Application number: 01965975.4
(22) Date of filing: 17.08.2001
(51) Int. Cl.: B05C 1/08

(54) **SUBSTRATE COATING AND APPARATUS FOR APPLYING THE SAME**
BESCHICHTUNG FÜR EIN SUBSTRAT UND VORRICHTUNG ZUM AUFTRAG DESSELBEN
REVETEMENT DE SUBSTRAT ET APPAREIL D'APPLICATION DE CE SUBSTRAT

(30) Priority: 18.08.2000 GB 0020279
(43) Date of publication of application: 21.05.2003
(73) Proprietor: MeadWestvaco Packaging Systems LLC, Stamford, Connecticut 06905 (US)
(72) Inventor: LEBRAS, Philippe, F-36000 Chateauroux (FR); TIMBAL, Olivier, F-36000 Chateauroux (FR)
(74) Representative: Hepworth, John Malcolm
(86) International application number: PCT/US2001/025751
(87) International publication number: WO 2002/016050

(56) References cited:
- EP-A- 0 542 190
- WO-A-98/24557
- DE-A- 19 542 097
- DE-U- 29 922 546
- US-A- 5 335 596
- US-A- 5 948 740
- US-A- 6 082 257

## Description

### Background of the Invention

This invention relates to a substrate coating. More particularly, the invention relates to a paperboard coating for food packaging. The invention also relates to an apparatus and method of applying the coating to a substrate.

When paperboard cartons are used for packaging food items, for example ready-meals or meat which contain liquid, a barrier in the form of a separate layer of material must be applied to the paperboard to ensure that the paperboard itself remains dry as far as possible and therefore retains its mechanical strength. The barrier also ensures that the liquid does not seep through the packaging. Preferably, the barrier should, additionally, be relatively impermeable to air in order to substantially prevent meat contained within the packaging from becoming discoloured, be insoluble when in contact with a wide range of solvents, be colour free, have substantially no odour, a high coefficient of friction and have hot-seal properties.

Most commonly, a plastics film layer is extruded or glued onto paperboard to make water or greaseproof packaging and can be used to package a wide range of foodstuffs including liquids. The extrusion process offers the fastest of the two coating methods and is the cheapest option for large production volumes, but requires high capital expenditure. The method is only viable if the process is to be carried out continuously. The gluing process has a lower capital outlay, but can only be carried out at lower speed and is therefore not cost effective for large production volumes. For both methods, the specific weight of the film that is applied is generally in the region of 20g/m². The film used is non-biodegradable, and is difficult to recycle because once the film has been adhered to the paperboard, it is problematic to separate the two again.

Additionally, a number of layers applied as a liquid have been proposed for use in food contact applications. US 5 776 619 to Shanton discloses a paperboard layer for use in forming rigid food containers. The layer comprises a base coat comprising a styrene acrylic polymer latex and pigment that is applied directly to the paperboard, and a top coat comprising a styrene acrylic polymer latex and pigment that is applied to the base coat. The layer seeks to improve grease, oil and cut resistance and enhance printing qualities.

US 4 097 297 to Keene discloses a nitrocellulose lacquer varnish that may be applied to either a clay coated or non-clay coated side of paperboard. To improve water and oil repellency, a fluorochemical surface tension modifier is added to the varnish.

WO-A-98 /24557 further discloses an apparatus for applying a coating to a substrate, wherein . a cylinder in the form of a rotatable or metering roller is provided onto which a liquid emulsion of the coating is introduced, a scraper for removing excess coating from the cylinder being also provided, as well as a second cylinder in contact with the first cylinder and arranged so as to transfer the coating from the first cylinder to the substrate; in this known arrangement, the scraper comprises one scraper blade and a coating reservoir whereby, in operation, minimal pressure is applied to the electrical steel strip to be coated in order to remove all surface irregularities therefrom.

### Summary of the Invention

The present invention seeks to meet the above criteria and overcome or at least mitigate the problems of the prior art.

According to a first aspect of the invention there is provided an apparatus for applying a coating to a substrate comprising a first cylinder onto which a liquid emulsion of the coating is introduced, a scraper for removing excess coating from the cylinder and a second cylinder in contact with the first cylinder and arranged so as to transfer the coating from the first cylinder to the substrate, wherein the scraper comprises two mutually opposed scraper blades and a coating reservoir wherein sufficient pressure is applied to the substrate so as to compress the substrate thereby to reduce the coating thickness and hence the coating weight ultimately applied to the substrate.

Preferably, pressure is applied to the substrate so as to compress the substrate by approximately 0.05 - 0.1 mm at working speeds.

According to an optional feature of the first aspect of the invention, the apparatus is flexographic apparatus.

According to an optional feature of the first aspect of the invention, the second cylinder is resilient. Preferably the second cylinder may be manufactured from EPDM or a photopolymeric flexographic sheet.

A second aspect of the invention provides a method of applying a coating to a substrate using the apparatus as claimed in any of claims 1 to 5 comprising the steps of:
i) applying a liquid emulsion of the coating to a first cylinder of a coating apparatus from a coating reservoir,
ii) removing excess coating from the first cylinder using a scraper blade associated with the coating reservoir,
iii) transferring the coating to a second cylinder in contact with the first cylinder, and
iv) transferring the coating to a substrate in contact with the second cylinder.

Preferably, the first cylinder of said apparatus is a honeycomb ceramic cylinder.

More preferably, the method may further comprise the step of drying the coating using a heating system.

More preferably, the method may further comprise the stage of applying pressure to the substrate so as to compress the substrate by approximately 0.05 - 0.1 mm at working speeds.

### Brief Description of the Drawings

The present invention is further described by way of example only, with reference to the accompanying drawings in which:
FIGURE 1 is a schematic side view of the apparatus for applying the coating to paperboard illustrating the reservoir;
FIGURE 2 is a side elevation of the scraper and scraper blades;
FIGURE 3 is a perspective view of one end of the scraper; and
FIGURE 4 is a view of the scraper illustrating the inlet and outlet pipes for the liquid coating.

### Detailed Description of the Preferred Embodiments

In general, prior art coatings that can be used in contact with moist foodstuff such as meat and ready-meals have been insufficiently resistant to water, leading to the foodstuff adhering to the paperboard, resulting in tearing of the board and likely unsightly discolouration of the board. Through extensive trials, a coating has been formulated that has been approved for direct contact with food and has achieved ISEGA certificate of conformity: recommendation XXXV BgVV for contact with moist, dry and greasy foodstuffs. Specifically, French DGCCRF (Direction Generale de la Consommation, de la Concurrence et de la Repression des Fraudes) approval has been obtained so that the formulation complies with European Council Resolution (96) 5. The DGCCRF in turn complies with EU directives 82/711, 93-8, 90-128, 92-39, 85-572 and the modifications to the 82/711 by 97/48/CE implemented on 29 July 1997. Furthermore, all compounds comprising the coating are on current EU non-toxic "positive lists", specifically resolution AP96/5 "Surface coatings intended to come into contact with foodstuffs" of the European Council and adopted by the Council of Ministers on 2 October 1996.

As part of the approval process, migration testing of the coating into foodstuffs (as simulated by a number of solvents e.g. distilled water, non-polar isooctane and polar ethanol) was carried out. The maximum migration permissible for each solvent is 10 mg/dm² or 60mg/kg of foodstuff over a seven day contact period.

The results of the testing of trays made from coated paperboard are summarised in table 1 below:

**Table 1**

| **Solvent** | **Contact Duration (days)** | **Temperature (°C)** | **Migration (mg/dm**^{**2**}**)** |
|---|---|---|---|
| Distilled water | 5 | 5 | 4.1 |
| Distilled water | 7 | 5 | 4.1 |
| Ethanol (95% conc.) | 3 | 5 | 2.8 |
| Ethanol (95% conc.) | 7 | 5 | 2.9 |
| Isooctane | 0.5 | 5 | 1.1 |

The next stage of the procedure for testing coating formulation procedure was the conducting of sensorial tests to ensure that odours from the coating do not taint foodstuffs with which they come into contact. The method followed is in accordance with French standard AFNOR XPV 09-0009 (September 1995) entitled "Method of evaluating foreign bodies migrating from packaging into foodstuffs" and NF V 09-013 (July 1983) "Sensorial analysis-triangular methodology test" (ISO 4120 equivalent). The test is conducted as follows: butter (which is used due to the ease with which it becomes tainted and retains flavours) is placed in contact with the coated board for a set period of 48 hours at 10°C. Two samples of exposed butter and an additional control sample are submitted to a taste panel and if more than one of the three panel members find the control butter, when assessed over a statistically significant number of tests, the test is failed. A coating formulation has been found that passes this test.

A voluntary final stage of the procedure is the specific migration test in which specific monomers and catalysts used in the coating are subjected to a migration test using a gas chromatograph. This test was developed to test migration into meat particularly. The formulation process has resulted in an acrylic coating formulation (not forming part of the present invention), one example of which is an oil in water emulsion. The emulsion comprises a liquid disperse phase and a continuous liquid phase. The liquid disperse phase comprises epoxide PE wax in a 5% concentration to provide the grease barrier properties. The formulation further comprises a wax dispersant, and preferably a surface tension modifier to aid the transfer of the coating from the cylinders and onto the paper by lowering the surface tension to less than 36-40 dynes/cm (the surface tension of the board) and an antifoaming agent. In this example, the formulation has a surface tension of 32 dynes/cm.

A second example dispenses with the epoxide PE wax to form an entirely water based solution of the coating without the PE wax.

The coating has excellent water resistance (Cobb test: <=1g/m² passing after one minute and <=5g/m² passing after 30 minutes) and grease resistance with a low permeability and low overall migration characteristics. A further advantage of the coating is that it is an oxygen barrier to increase the shelf life of the foodstuff held by the package.

Furthermore, the coating is substantially non-adhesive and colour free, is insoluble over a wide range of different simulating solvents, has a low odour and is non-delaminating but does have some relative adhesion for foodstuffs such as turkey. This may be achieved by the addition of a blocking agent to the formulation. Some relative adhesion is advantageous as this permits cartons made from the coated paperboard and containing foodstuffs to be placed on shelving angled toward purchasers of the foodstuffs whilst maintaining the foodstuffs in a desired position within the carton. This in turn enhances the presentation and marketability of the foodstuffs.

The coating is also advantageously heat sealable. A coating to coating seal can be achieved at a temperature of 150°C and a pressure of 2 bars for 2 seconds. For a coating to board seal, a temperature of 160°C and a pressure of 3 bars should be maintained for 5 seconds. The fact that any attempt to tear board coated using the above coating results in the delamination of the board indicates that a good seal is achieved.

In one class of embodiments, the coating is absorbed partially by the substrate, for example the coated board.

Turning to Figure 1 there is shown apparatus 10 for applying a coating to a substrate such as paperboard 20 using a flexography process. A liquid emulsion or solution of the coating is applied to the surface of an anilox cylinder 12. In a preferred embodiment, a ceramic honeycomb cylinder permits an accurate proportion of the coating to be transferred to the blanket cylinder 16. The honeycombs are preferably 35 microns in depth, with there being 90 cells/linear cm giving an effective capacity of 11-14 cm³/m². For the preferred coating, 6g/m² is transferred in one pass (40% of the theoretical volume) with a 60° engraving angle. This type of anilox cylinder 12 is used as this enables an increased amount of the coating to be carried by the cylinder. A scraper 14 removes any excess coating before the coating is transferred from the anilox cylinder 12 to the blanket cylinder 16. The cylinder 16 is advantageously made of resilient material such as butyl, EPDM (ethylene propylene diene methylene), nitrile or silicone rubber. Preferably however, EPDM or a Cyrel^{RTM} type photopolymeric flexographic sheet having a hardness of approximately 50-80° shore is used.

Referring in particular to Figures 2, 3 and 4 the scraper is illustrated in more detail. It can be seen from Figure 2 that the scraper 14 comprises upper and lower scraper blades 28 and 30 mounted on a coating reservoir portion 32. The scraper 14 is, in this embodiment, adjustably mounted in relation to the anilox cylinder 12 by a pair of locating holes 40a and 40b that engage corresponding fingers (not shown) provided on a frame that supports the cylinders. Adjustment means for adjusting the position of the scraper in relation to the cylinder 12 is provided. In this embodiment, a pair of pressure adjusting screws 36a and 36b is provided .

Increasing the pressure between the scraper blades 28, 30 and the anilox cylinder 12 reduces the coating thickness applied on the anilox cylinder 12 and hence the coating weight ultimately applied to the paperboard 20. The screws may be used in conjunction with pressure gauges that are calibrated such that screw adjustments may be directly related to the thickness of coating to be applied. In a particularly preferred embodiment, the method of applying pressure is automated as part of an overall control system for the apparatus (not shown).

It can also be seen from Figures 2 and 3 that suitable sealing means, for example resilient seals 34a and 34b, formed from rubber or similar materials, are provided at each end of the reservoir 32 to prevent, or at least substantially minimise coating leakage.

Referring now to Figure 4 which shows a rear view of the scraper 14, the infeed apertures 38a and 38b and outfeed aperture 42 for the liquid coating can be seen. In this embodiment, pipes (not shown) feed the liquid coating into the reservoir 32 at each end thereof preferably from a peristaltic pump. Any excess coating then exits the reservoir at the centre through outfeed aperture 42 and is recycled. A closed or open loop coating supply system may be employed. It is preferred that a closed system is used as this substantially prevents contact between the coating and the atmosphere.

Turning back to Figure 1, anilox cylinder 12 is arranged to be in contact with blanket cylinder 16, the rotation thereof transferring the coating from the anilox cylinder 12 to the blanket cylinder 16. The thickness of the coating is adjusted by changing the velocity of one of the anilox cylinder or blanket cylinder relative the other. A controller is used to control the rotational velocities of each cylinder. The linear velocity of the anilox cylinder 12 is preferably 1.05 to 1.10 times greater than the linear velocity of the blanket cylinder 16. This enables a thick layer of coating to be more evenly applied to the paperboard 20. Paperboard, either in the form of a continuous sheet or in discrete pieces 20 as shown, is fed into the apparatus by a first conveyor belt 22 running at the same linear velocity as the blanket cylinder 16. A force is applied by the apparatus to the anilox cylinder 12, in a direction X, the load being transferred via the blanket cylinder 16 such that the paperboard 20 is typically compressed by approximately 0.05 - 0.1 millimetres at normal running speeds and the coating is transferred to the paperboard 20 and in greater amounts than would be possible using an off-set process. The above described arrangement ensures that an even layer of the liquid emulsion is applied to the paperboard 20. An impression roller 18 is provided underneath the paperboard 20 so as to guide the paperboard past the blanket cylinder. Where it is necessary to blank areas of paperboard from printing, portions of the blanchet cylinder 16 may be recessed so as not to pick up the coating from the anilox cylinder 12.

The coated paperboard is then preferably transferred by a second conveyor 24 to a heater 26 in direction Y. This ensures that the coating is dry before the paperboard 20 is processed further, or is stored. A particularly preferable heating system comprises a hot air flow at a temperature of approximately 180°C used in addition to infrared radiation for at least two seconds. It is preferable that the temperature should reach at least 85°C on the support conveyor 24. In a particularly preferred arrangement, four 6kW infrared lamps (not shown) are used that emit radiation in a spectrum of 500 nm to 2000 nm wavelength to give a good coating surface whilst avoiding "orange skin" effects. A long drying station may be used to avoid off-setting as this provides sufficient time for the coating to dry before the paperboard 20 is stacked or rolled up.

The coating is partially absorbed into the paperboard, with any remainder forming a layer on the surface thereof. The degree of absorption depends upon, amongst other factors, the characteristics of the paperboard and the interval between applying the coating and the paperboard entering the heater 26.

To ensure that a sufficiently thick and even layer of the coating is provided on a surface of the paperboard 20 in some classes of embodiment, a second coating is advantageously applied to the paperboard by a similar apparatus as described above. Thus, a thicker coating for example 9g/m² can be obtained. In certain classes of embodiment, the second layer has different properties from the first, and the two layers have complementary properties so as to achieve the desired result. For example, the first layer may include a pigment.

For the coated board to be considered biodegradable "mono" material according to German standards (Töpfer regulation and the Verpackungs-Verordnung), the coating must comprise less than 5% of the board weight. Therefore, for a standard 300 g/m² board, the coating weight must be lower than 15 g/m². Furthermore, in order for the finished board to be considered recyclable it is necessary for the coating weight to be less than 10 g/m². However, the preferred total coating weight applied by the above apparatus is in the range of 6-7 g/m² dry.

In other classes of embodiment, dependent upon the actual set-up of the apparatus and the properties of the coating, a single pass with a longer drying time may be sufficient. The chances of achieving a coating weight of 6-7 g/m² in a single pass are enhanced if the ceramic "honeycomb" anilox cylinder 12 is used.

Thus, there is provided a recyclable and repulpable coated substrate. The coating is in the range of 3 to 10g/m² and comprises one or more coatings, which formed a pinhole free continuous coating resistant to water.

The above described apparatus is generally capable of coating 130-150 metres of paperboard per minute by the abovementioned continuous application process. Following coating, the paperboard is cut, creased and glued as necessary. If aseptic packaging is required, the paperboard can then be treated with a hydrogen peroxide solution or other suitable antimicrobial agent.

It should be understood that numerous changes may be made within the scope of the invention which is defined by the appended claims. For example, alternative substrates such as linerboard or paper may be used.

## Claims

1. Apparatus (10) for applying a coating to a substrate comprising a first cylinder (12) onto which a liquid emulsion of the coating is introduced, a scraper for removing excess coating from the cylinder (12) and a second cylinder (16) in contact with the first cylinder (12) and arranged so as to transfer the coating from the first cylinder to the substrate, wherein the scraper (14) comprises two mutually opposed scraper blades (28, 30) and a coating reservoir (32) wherein sufficient pressure is applied to the substrate so as to compress the substrate thereby to reduce the coating thickness and hence the coating weight ultimately applied to the substrate.

2. Apparatus (10) according to claim 1 which is flexographic apparatus.

3. Apparatus (10) according to claim 1 or claim 2 wherein the second cylinder (16) is resilient.

4. Apparatus according to claim 3 wherein the second cylinder (16) is manufactured from EPDM or a photopolymeric flexographic sheet.

5. Apparatus according to any one of claims 1 to 4 wherein the first cylinder (12) is a honeycomb ceramic cylinder.

6. A method of applying a coating to a substrate using the apparatus as claimed in any of claims 1 to 5 comprising the steps of:
i) applying a liquid emulsion of the coating to a first cylinder (12) of a coating apparatus from a coating reservoir (32),
ii) removing excess coating from the first cylinder (12) using the scraper blades (28, 30) of the scraper (14) associated with the coating reservoir (32),
iii) transferring the coating to a second cylinder(16) in contact with the first cylinder (12), and
iv) transferring the coating to a substrate in contact with the second cylinder (16).

7. A method according to claim 6 wherein pressure is applied to the substrate so as to compress the substrate by approximately 0.05 - 0.1 mm at working speeds.

8. A method according to claim 6 or claim 7 further comprising the step of drying the coating using a heating system (26).

## Patentansprüche

1. Vorrichtung (10) zum Aufbringen eines Belages auf ein Substrat, wobei die Vorrichtung einen ersten Zylinder (12) umfasst, in den eine flüssige Emulsion des Belages eingeführt wird, einen Abstreicher zum Entfernen überschüssigen Belages von dem Zylinder (12), einen zweiten Zylinder (16), der in Kontakt mit dem ersten Zylinder (12) steht und derart angeordnet ist, dass der Belag von dem ersten Zylinder auf das Substrat überführt wird, wobei der Abstreicher (14) zwei gegenüberliegend angeordnete Abstreicher-Blätter (28, 30) umfasst, ferner ein Belag-Reservoir (32), wobei hinreichender Druck auf das Substrat aufgebracht wird, um das Substrat zu komprimieren, um so die Dicke des Belages zu reduzieren und damit das Belagsgewicht, das letztendlich auf das Substrat aufgebracht wird.

2. Vorrichtung (10) nach Anspruch 1, wobei die Vorrichtung eine Flexodruck-Vorrichtung ist.

3. Vorrichtung (10) nach Anspruch 1 oder 2, wobei der zweite Zylinder (16) nachgebend ist.

4. Vorrichtung nach Anspruch 3, wobei der zweite Zylinder (16) aus EPDM oder einem photopolymerischen Flexodruck-Blatt hergestellt ist.

5. Vorrichtung nach einem der vorhergehenden Ansprüche 1 bis 4, wobei der erste Zylinder (12) ein Waben-Keramikzylinder ist.

6. Verfahren zum Aufbringen eines Belages auf ein Substrat unter Verwendung einer Vorrichtung gemäß einem der vorstehenden Ansprüche 1 bis 5, wobei das Verfahren folgende Schritte umfasst:
i) Aufbringen einer flüssigen Emulsion des Belages auf einen ersten Zylinder (12) einer Vorrichtung zum Aufbringen eines Belages aus einem Belag-Reservoir (32),
ii) Entfernen überschüssigen Belages von dem ersten Zylinder (12) durch Verwenden der Abstreicher-Blätter (28, 30) des Abstreichers (14), der dem Belag-Reservoir (32) zugeordnet ist,
iii) Überführen des Belages auf einen zweiten Zylinder (16), der in Kontakt mit dem ersten Zylinder (12) steht, und
iv) Überführen des Belages auf ein Substrat, das in Kontakt mit dem zweiten Zylinder (16) steht.

7. Verfahren nach Anspruch 6, wobei Druck auf das Substrat aufgebracht wird, um so das Substrat um etwa 0,05-0,1 mm bei Arbeitsgeschwindigkeit zu komprimieren.

8. Verfahren nach Anspruch 6 oder 7, das weiterhin den Schritt des Trocknens des Belages unter Verwendung eines Heizsystems (26) umfasst.

## Revendications

1. Appareil (10) pour appliquer un revêtement sur un substrat comprenant un premier rouleau (12) sur lequel est introduite une émulsion liquide du revêtement, un racleur pour supprimer du rouleau (12) le revêtement en excès, et un deuxième rouleau (16) en contact avec le premier rouleau (12) et adapté pour transférer le revêtement du premier rouleau au substrat, le racleur (14) comprenant deux lames de racleur mutuellement opposées (28, 30) et un réservoir de revêtement (32) dans lequel une pression suffisante est appliquée au substrat pour comprimer le substrat afin de réduire l'épaisseur du revêtement et donc le poids du revêtement finalement appliqué au substrat.

2. Appareil (10) selon la revendication 1 qui est un appareil pour impression flexographique.

3. Appareil (10) selon la revendication 1 ou 2, dans lequel le deuxième rouleau (16) est résilient.

4. Appareil (10) selon la revendication 3, dans lequel le deuxième rouleau (16) est fabriqué à partir d'EPDM ou d'une plaque de photopolymère flexographique.

5. Appareil (10) selon l'une quelconque des revendications 1 à 4, dans lequel le premier rouleau (12) est un rouleau en céramique en nid d'abeilles.

6. Procédé d'application d'un revêtement sur un substrat utilisant l'appareil de l'une quelconque des revendications 1 à 5, comprenant les étapes consistant à :
i) appliquer une émulsion liquide du revêtement sur un premier rouleau (12) d'un appareil de revêtement depuis un réservoir de revêtement (32),
ii) supprimer du premier rouleau (12) le revêtement en excès en utilisant les lames de racleur (28, 30) du racleur (14) associé au réservoir de revêtement (32),
iii) transférer le revêtement sur un deuxième rouleau (16) en contact avec le premier rouleau (12), et
iv) transférer le revêtement sur un substrat en contact avec le deuxième rouleau (16).

7. Procédé selon la revendication 6, dans lequel on applique une pression sur le substrat afin de comprimer le substrat d'environ 0,05 à 0,1 mm aux vitesses de travail.

8. Procédé selon la revendication 6 ou 7, comprenant en outre l'étape consistant à sécher le revêtement en utilisant un système de chauffage (26).
